

# UNITED STATES PATENT OFFICE.

RICHARD GREULICH, OF LUDWIGSHAFEN-ON-THE-RHINE, GERMANY, AND HERBERT LICKFETT, OF RJUKAN, TELEMARKEN, NORWAY, ASSIGNEES TO THE FIRM OF GEBRÜDER GIULINI, G. M. B. H., OF LUDWIGSHAFEN-ON-THE-RHINE, GERMANY.

## MANUFACTURE OF METAL NITROGEN COMPOUNDS.

1,268,240.

Specification of Letters Patent.

Patented June 4, 1918.

No Drawing.

Application filed November 28, 1913. Serial No. 803,572.

*To all whom it may concern:*

Be it known that we, RICHARD GREULICH, chemist, a subject of the King of Saxony and the German Emperor, and HERBERT LICKFETT, chemist, a subject of the King of Prussia and the German Emperor, residing at Ludwigshafen - on - the - Rhine, Bayernstrasse 34, Kingdom of Bavaria, German Empire, and Rjukan, Telemarken, Kingdom 10 of Norway, respectively, have invented a new and useful Improvement in the Manufacture of Metal Nitrogen Compounds; and we do hereby declare the following to be a full, clear, and exact description of the same.

15 It is known that in the production of aluminium nitrid by heating a mixture of alumina and carbon in the presence of nitrogen, the temperature of formation can be lowered by the addition of a basic metal 20 oxid, or hydroxid, such as lime, baryta and the like or by the addition of salts of such metals. In practice it has however been found that the amount which can be used of such additional substance is too small to 25 accelerate, or facilitate, to any marked degree, the formation of the nitrid and, even with from 2 to 6 per cent. of the additional substance, great difficulties arise in the practical carrying out of the process, as the mixture sinters and melts and the walls of the 30 vessels are highly attacked and the nitrogen does not obtain proper contact with the sintered, or molten, mass, and, the yield of aluminium nitrid is very small.

35 These objections are greater when, in order to accelerate the reaction, larger amounts of the additional substance are used as then the mass fuses and forms a solid slag and entirely prevents the passage 40 of the nitrogen, so that practically no nitrid is formed.

It has been proposed to prevent, or reduce, this slagging in various ways; for instance, in the specification of Serpels German Patent No. 235,669, it is proposed to first heat a mixture of 40 parts of alumina, 4 parts of baryta and 12 parts of carbon without supplying nitrogen and then to powder the cooled slag thus produced and then in a second operation to heat the powdered slag in a current of nitrogen together with alumina. This process presents great difficulties in practice, as, owing to the slagging of the

product, the walls of the vessels are highly attacked, and injured and the division of 55 the process into two phases causes waste of time and is expensive and the process cannot be carried on continuously.

It has been proposed to overcome the objections by adding a large excess of carbor, 60 and it is possible to decrease the slagging by the use for instance of a quantity of carbon in excess equal to twenty times the quantity theoretically required but the product obtained is contaminated with a considerable amount of carbid and carbon which is not suitable to a manufacture of alumina, etc., and further, the process is not economical, as an enormous amount of carbon is heated uselessly without increasing the yield 70 of nitrid.

We have found that it is possible to successfully use, in the manufacture of metal nitrogen compounds as nitrids, for instance aluminium nitrid, large amounts of additional substances, such as a basic metal oxid, or hydroxid, or a salt, for accelerating the reaction, so as to control and regulate the velocity of reaction according to requirements and to avoid slagging and thereby 75 allow the absorption of nitrogen to be uniform and cause the vessels to last longer, if a mixture of alumina, or alumina-containing substance and carbon with any desired amount of metal oxid or the like, be heated 80 in a vessel (such for instance as a tube) which is formed of carbon, or which is provided internally with a covering or coating or lining of carbon, as then not only will the walls of the vessel be protected but coalescing and slagging together of the substances employed will be prevented.

This invention in contradistinction to the known processes enables the amount of the metal oxid, or other additional substance, to 95 be added to the mixture of alumina and carbon, to be varied as desired so that the greatest amount of such additional substance desired can be used to accelerate the reaction while no melting of the mass occurs, it 100 remaining so porous as to allow the proper passage of the nitrogen through the mass. In consequence the yield of aluminium nitrid is considerably increased, as compared with the earlier processes while the large proportion of the additional substance used con-

siderably lowers the temperature of formation of the nitrid, which is obtained in a condition better adapted for subsequent treatment. Caking of the particles of material together and adherence to the walls of the vessel are prevented also when coarse pieces of material are employed.

We have found that a vessel, or tube, with an inner surface of carbon or such a tube 10 of carbon especially if it is as pure as possible (such for instance as the carbon used for electrodes) is not chemically attacked, or destroyed, by the incandescent mass therein. The presence of oxid of iron, 15 titanium, silicon, or similar matters which may occur in the initial material, such, for instance, as beauxite, is not injurious and the mechanical wear is very small, even when coarse pieces of material are employed.

20 The process according to this invention can be carried out as follows; but we do not limit ourselves to this example.

Alumina, or alumina-containing material is mixed with coal, or other kind of carbon, 25 or carbonaceous matter, and any suitable large proportion of a basic metal oxides (for instance  $\text{CaO}$ ,  $\text{BaO}$ ,  $\text{MgO}$ ) or of a salt (for instance  $\text{Na}_2\text{CO}_3$ ,  $\text{K}_2\text{CO}_3$ ,  $\text{CaCO}_3$ ,  $\text{BaSO}_4$ ) and the mixture is placed in a vessel such 30 as a retort, or tube, or the like of refractory material, for example burnt fire-clay, which is heated from the outside while nitrogen is passed through. The inner wall of the said vessel, tube, or the like, is coated entirely, 35 or only along the firing zone, with a layer of carbon such as graphite, or the like. For example such a coating of firmly adherent graphite can be readily obtained by raising coal to incandescence in the vessel, tube, or 40 the like, of refractory material from which air is excluded. In this way a firm coating of carbon is deposited on the inner wall of the vessel, tube, or the like. Instead of coating the vessel, tube, or the like, with a 45 layer of graphite or other form of carbon, vessels, tubes, or the like, of burnt fire-clay may be provided with an inner tube of coal, or other form of carbon which, for preventing loss of heat, should fit as closely as practicable, the outer vessel, tube, or the like.

It is advantageous to carry out the process in a continuous manner, by supplying the mixture of alumina, carbon, and any suitable large proportion of additional substance 55 and the nitrogen to the vessel, tube, or the like, having an interior of carbon the nitrid formed being tapped off from below.

From the foregoing description it will be

readily understood that the invention can be similarly applied to the manufacture of 60 nitrids other than aluminium nitrid and also to the manufacture of cyanids and the like by suitable selection of the initial materials.

It has been proposed for heating mixtures of aluminous material and carbon, but without additions facilitating the absorption of nitrogen, to use carbon tubes as conductors for electricity, in order to vaporize the impurities present in the aluminous material, especially silica, alkaline earths and alkalis, 70 for which high temperatures available by electricity. The present invention refers exclusively to the manufacture of nitrids by means of mixtures of the initial material, carbon and any suitable large proportion 75 of additions facilitating the absorption of nitrogen leaving out of account the small quantities of impurities being contained in the initial material. The use of such mixtures has been also proposed, but not in combination with carbon vessels. We do not claim the said features separately but only the combination of the two features.

Having now particularly described and ascertained the nature of our said invention; 80 and in what manner the same is to be performed, we declare that what we claim is—

1. In the manufacture of nitrogen compounds of metals, the step which consists in heating a mixture of compounds of the 90 metal with substances accelerating the absorption of nitrogen thereby, in a carbon lined vessel, in the presence of nitrogenous gases, and to a temperature below the sintering temperature of the mixture.

2. In the manufacture of nitrogen compounds of metals in a carbon lined vessel, mixing the initial compound of the metal with such amount of substances accelerating the absorption of nitrogen that a deleterious 100 slagging would result if the retort were not carbon lined; conducting the mixture into such a vessel; and heating the mixture while therein, by exteriorly heating said vessel, to a temperature below the sintering temperature of the mixture, and in the presence of nitrogenous gases.

In testimony whereof, we have signed our names to this specification in the presence of two subscribing witnesses.

RICHARD GREULICH.  
HERBERT LICKFETT.

Witnesses:

BRUNO BOHM,  
L. S. BERGEE.